

T. SLOPER.

BEADED STRIP OF METAL AND THE PROCESS OF ROLLING THE SAME.

APPLICATION FILED APR. 14, 1919.

1,343,753.

Patented June 15, 1920.

2 SHEETS—SHEET 1.

*Fig. 1.*



*Fig. 1.*

*Fig. 2.*



*Fig. 3.*



*Fig. 4.*



*F<sup>2</sup>*

*C*

*F<sup>1</sup>*

*C<sup>4</sup>*

*Fig. 5.*

*C<sup>4</sup>*



Thomas Sloper,  
Inventor,  
By Russell, Byers & Palmer  
Attest.

T. SLOPER.

BEADED STRIP OF METAL AND THE PROCESS OF ROLLING THE SAME.

APPLICATION FILED APR. 14, 1919.

1,343,753.

Patented June 15, 1920.

2 SHEETS—SHEET 2.

Fig. 6



Fig. 7



Fig. 8



Thomas Sloper  
J. Smith  
by Bettsell, Beynes & Parsons  
Atty.

# UNITED STATES PATENT OFFICE.

THOMAS SLOPER, OF DEVIZES, ENGLAND.

## BEADED STRIP OF METAL AND THE PROCESS OF ROLLING THE SAME.

1,343,753.

Specification of Letters Patent. Patented June 15, 1920.

Application filed April 14, 1919. Serial No. 289,817.

To all whom it may concern:

Be it known that I, THOMAS SLOPER, a subject of the King of England, residing at Devizes, Wiltshire, England, have invented 5 certain new and useful Improvements in Beaded Strips of Metal and Processes of Rolling the Same, of which the following is a specification.

This invention is for improvements in or 10 relating to beaded strips of metal and to the process of rolling the same and is particularly applicable to the rims of wheels for aircraft where lightness is of considerable importance, and which wheels are to 15 receive pneumatic tires.

It is common practice to thicken the edge 20 of the over-turned lip which engages the bead of the tire, by folding the edge of the metal strip from which the rim is made over on to itself thus making it of double thickness at the lips.

For this purpose it is necessary to employ 25 steel which is very soft, otherwise it will crack where it is folded, and the thicker the metal the more liable it is to crack.

The object of the present invention is to 30 enable the edges of a strip to be thickened without folding them back in this manner, so that a harder steel can be employed and 35 a stiffer rim or strip produced for a given weight.

It has before been proposed to provide a 40 strip of steel for rim-making with thickened edges by hot rolling to produce a flat strip with the said thickened edges, but the strip so produced varies more or less in width.

The process for producing a strip with 45 thickened edges according to this invention consists in (a) passing a flat strip between rollers to bend it into channel-form and (b) passing it between other rollers which maintain the channel-form, but are shaped to crush the upstanding edges inward and laterally outward whereby such edges are thickened; the space between the rollers is preferably so dimensioned that it is entirely filled by the metal thus treated.

In the accompanying drawings:—

50 Figure 1 is a longitudinal section through part of the first pair of operating-rolls with the metal between them as arranged for making a wheel-rim strip;

55 Fig. 2 is a similar view of the second pair of operating-rolls;

Fig. 3 is a similar view of the third pair;

Fig. 4 is a similar view of the fourth pair of rolls;

Fig. 5 shows a transverse section through a completed wheel-rim whereof the thickened edges are constructed according to this invention;

Fig. 6 is a longitudinal section through part of the first pair of operating rolls for producing a beaded strip according to this invention, not intended for wheel-rims, the strip moreover being shown in position between the rolls;

Fig. 7 is a similar view of the second pair of rolls for the same strip;

Fig. 8 is a similar view of the third pair of rolls for the same strip, and

Fig. 9 shows the completed strip flattened out.

The same letters indicate the same parts throughout the drawings.

The rolls for producing the thickened edges are of simple construction as the required shapes can all be obtained by properly-shaped steps at the ends of the rolls. 50 In Fig. 1, the upper roller A enters the lower roller B and has an inclined step at A<sup>1</sup>; the lower roller has a correspondingly inclined step. The metal strip C is thus kept flat across the greater part of its width but is bent up at the edges providing an angle C<sup>1</sup>. The strip is passed from the rollers A B to the rollers D D<sup>1</sup> shown in Fig. 2. In these rollers, not only an oblique step D<sup>2</sup> is provided, but also a vertical step D<sup>3</sup>, so 55 that the metal C has a second angle formed at C<sup>2</sup> which brings the part that lies beyond the angle C<sup>1</sup> into a perpendicular position relatively to the main body of the strip.

In the third pair of rollers, the roller E which co-operates with the roller E<sup>1</sup>, is provided with steps E<sup>2</sup> and E<sup>3</sup> which lie at the same angles as the steps D<sup>2</sup> D<sup>3</sup> but the step E<sup>3</sup> is shortened and widened, with the result 100 that the metal at each edge of the strip C is crushed inward toward the main body of the metal and allowed to swell laterally outward providing the thickened edges C<sup>3</sup>.

In the fourth pair of rolls, this crushing 105 is carried a step farther, the rolls F and F<sup>1</sup> providing a still shorter step at F<sup>2</sup>, the width of the space provided by this step being still wider than the corresponding step in the rolls E E<sup>1</sup> so that the edges of the 110 strip C are still farther crushed inward and swelled laterally as shown at C<sup>4</sup>,

To insure that the thickening of the metal should take place at the desired position the space between the rolls should be so dimensioned that it is entirely filled by the metal 5 as it passes between them except where the increase in thickness is desired.

It is found that by this process the thickening can be effected without heating and can be carried out uniformly and to any desired extent. 10

Preferably the strip for treatment according to this process has sheared edges to insure uniformity in the width.

The further shaping of the rim may be effected in known manner and constitutes no part of the present invention. The complete rim is shown in Fig. 5, where the thickened edges C<sup>4</sup> are shown bent inward to the position they assume for receiving the tire. The rim shown is tied in laterally by ties C<sup>5</sup> to prevent outward displacement of the edges under pneumatic pressure. 20

An important practical feature of the present invention lies in the fact that the edges of the rim which are to be crushed in are brought to such a position that they lie radially to the axes of the rollers when they are being crushed inward to thicken them. 25

30 Figs. 6 to 9 show the process and means for producing a flat strip having beaded or thickened edges, which edges are produced in the same manner as already described by crushing the edges inward, this strip, however, being serviceable for any desired purpose and not restricted in its use to wheel-rims. The strip in this case is not bent angularly at any point but is bent into U-shaped channel-form, as shown in Fig. 35 6, the rollers G and G<sup>1</sup> being shaped to give this form to the strip.

In Fig. 7, the rollers G<sup>2</sup> and G<sup>3</sup> are shaped still to give the same general form and to fit the strip at all parts except at the edges 45 H where space is allowed so that the edges are crushed inward and spread laterally as shown in the figure.

In Fig. 8, the rollers G<sup>4</sup> and G<sup>5</sup> are shaped to still further crush the edges H<sup>1</sup>. The strip is then finished and can be made into 50 any desired form or flattened out as shown at H<sup>2</sup>, Fig. 9, the flattening being effected by passing it between other rollers as will be readily understood.

What I claim as my invention and desire 55 to secure by Letters Patent is:—

1. The method of forming a shape having a reinforced flange, comprising the steps of rolling a blank and engaging the main portion of the body thereof between 60 the rolls of a roll pass to retain it against lateral displacement, and upsetting the edge of the blank in said pass to increase the thickness thereof, substantially as described.

2. The method of forming a metal shape 65 having a reinforced flange, comprising the steps of rolling an angular blank and engaging the main portion of the body thereof between the rolls of a roll pass to retain it against lateral displacement, and upsetting the edge of the blank to increase the thickness thereof, substantially as described. 70

3. The method of forming a shape having reinforced flanges, comprising the steps of rolling a channel shaped blank and engaging the main portion of the body thereof 75 between the rolls of a roll pass to retain it against lateral displacement, and upsetting the edges of the blank while traveling through said pass to increase the thickness 80 thereof, substantially as described.

4. The method of producing thickened edges on a metal strip, which comprises bending the strip into channel form having substantially vertical sides, tightly engaging 85 said member throughout the main portion thereof while leaving a portion of the vertical sides free, and then vertically upsetting the free portion of said sides to simultaneously decrease the height thereof and 90 increase the thickness, substantially as described.

In testimony whereof I affix my signature.  
THOMAS SLOPER.